

Aug. 30, 1960

H. M. HARTZBAND ET AL

2,951,022

PREPARING LUBRICATING OILS USING RADIATION

Filed Jan. 24, 1957



FIG. II



FIG. I

Harry M. Hartzband

Barry L. Tarmy Inventors

Robert B. Long

By *L. a. Steinbeck* Attorney

1

2,951,022

PREPARING LUBRICATING OILS USING  
RADIATION

Harry M. Hertzband, Westfield, Barry L. Tarmy, Cranford, and Robert B. Long, Wanamassa, N.J., assignors to Esso Research and Engineering Company, a corporation of Delaware

Filed Jan. 24, 1957, Ser. No. 636,066

7 Claims. (Cl. 204—154)

The present invention is concerned with a continuous process for producing high-quality lubricating oils from paraffinic feed stocks through the use of high energy ionizing irradiation.

In brief compass this invention proposes a process comprising irradiating a predominantly paraffinic feed boiling in the range of about 100 to 700° F. with high energy ionizing radiation at a temperature in the range above the pour point of the feed (ca. 50° F.) to 700° F. until at least  $5 \times 10^{-3}$  kilowatt-hours/pound (kw. h./lb.) of radiation have been absorbed to obtain a conversion of at least 1 wt. percent of the feed per pass. The material so irradiated is then separated to recover an intermediate boiling range (ca. 750/950° F.) lubricating fraction having a viscosity in the range of 35 to 70 SSU at 210° F., although it can be higher, and a viscosity index (V.I.) above 120. The material boiling below this intermediate boiling range fraction is recycled to the radiation zone.

It has now been found that the product obtained by irradiating a paraffinic feed material shows a rather unique variation of viscosity index with viscosity, as compared with conventional lubricating distillates. As expected, the irradiated material increases in viscosity as the boiling point goes up. The viscosity index for irradiated materials reaches, however, a maximum at some intermediate viscosity. This is not true for conventional lubricating distillates as they show a relatively flat but decreasing viscosity index with increasing viscosity.

The present invention incorporates this surprising finding into a continuous process typified by recovery of a high V.I. product. The process of this invention also embodies several other important features.

The drawings attached to and forming a part of this specification, and the following explanation and examples, will serve to make this invention clear. In the drawings, Figure I presents schematically the process of this invention, and Figure II presents a graph illustrating the unexpected relationship between viscosity and viscosity index of the irradiated product.

The feed material for the present invention boils in the range of 100 to 700° F. It usually has a viscosity below 35 SSU at 210° F., and is not generally considered a material suitable for lubricating purposes. The feed material used is predominantly paraffinic. By this is meant it contains at least 75 wt. percent of paraffinic hydrocarbons. It is preferably low in aromatics, both single and condensed ring, i.e., the feed material contains less than 5 wt. percent aromatics. It may contain some olefins and naphthenes within the boiling range, but preferably these do not exceed about 25 wt. percent. The feed stock may also contain up to 20 wt. percent of low molecular weight, or light, C<sub>2</sub>—C<sub>6</sub> unsaturates such as ethylene, and/or some light, C<sub>1</sub>—C<sub>5</sub> saturates such as propane.

The feed stock can be obtained from any convenient source. It can be obtained directly from crudes by distillation and/or from other hydrocarbon materials such

2

as Fischer-Tropsch synthesis products, shale oils, and refinery stream such as catalytic cycle stocks. In most instances it is desirable to treat the feed material to meet the above limitations. This may be done by such means as extraction with sulfur dioxide or furfural, by precipitation such as with propane, by adsorption as with silica gel, by dewaxing, by crystallization, besides by distillation or fractionation, and combinations thereof, all of which methods are known in the art.

With reference to the drawing, the above described feed material is introduced by line 1 into an irradiation zone 2, to be treated according to this invention with high energy ionizing radiation. By high energy ionizing radiation is meant radiation from terrestrial sources consisting of photons having a wave length less than 50 Å., such as gamma and X-rays, rapidly moving charged or uncharged particles of an atomic or subatomic nature having an energy above 30 ev., such as alpha particles and beta rays, and neutrons, the radiation being of sufficient intensity such that the dose rate is at least  $1 \times 10^{-3}$  kw. h./lb./hr. This excludes radiation such as cosmic and ultraviolet. It is much preferred to use radiation comprising neutrons such as that obtained from a nuclear reactor, so that at least 30% of the energy received is obtained from the neutrons.

The feed material is irradiated to an extent sufficient to obtain the product characteristics described below. The material receives a dose of at least  $5 \times 10^{-3}$  kw. h./lb., based on fresh feed, and over-irradiation is to be avoided. The maximum amount of radiation used should be under 1 kw. h./lb., based on fresh feed. The rate of irradiation is somewhat important. If it is too low, the excited molecules are "too diluted" to effectively react; and if over-extensive, cracking predominates to polymerization. While the invention is operable in the range of 1 to  $50 \times 10^{-3}$  kw. h./lb./hr., best results are obtained in the range of 4 to 8.

The irradiation can be obtained from any convenient source such as charged particle accelerators, e.g., Van de Graaff generators and Betatrons; from nuclear reactors, e.g., atomic piles; waste materials from nuclear reactors e.g., spent fuel elements; and materials made radioactive by insertion into a nuclear reactor, e.g., cobalt 60. The use of an atomic pile wherein mixed gamma and neutron irradiation is obtained is much preferred. This means that the feed material should be substantially free (contain less than 0.5 wt. percent) of non-hydrocarbon materials that may become radioactive by neutron irradiation, such as sulfur and chlorine.

The feed material is exposed to the irradiation in any convenient manner. For example, if an atomic pile is used, the feed material can simply be flowed through suitable conduits or pipes, in, around, and through the pile. The position of the feed material containing conduits within the pile partially determines the intensity of irradiation.

The pressure during irradiation is not too important, it generally being sufficient to maintain condense phase conditions. Pressures used can range from 0 to 4000 p.s.i.g., or above. The temperature is important. While this invention is operable at temperatures up to about 700° F., best results are obtained at temperatures in the range of 300 to 600° F. Excessively high temperatures result in a loss of product to cracking reactions, and low temperatures may undesirably decrease the reaction rate besides undesirably affecting the product characteristics.

When using pile irradiation, which comprises neutrons, it may be desirable to add to the feed isotopes that, upon capture of a neutron, admit highly energetic secondary irradiation. Thus, boron 10 and/or lithium 6 can be added to the feed material to create highly ionizing alpha

particles. Cadmium 113 can be used to create highly energetic gamma rays from the neutrons. These materials can exist in amounts in the range of 0.001 to 1 wt. percent as soluble compounds, as discrete subdivided solids, or can be distended on the surface of radiation inert solids.

As previously indicated, the irradiated material is withdrawn by line 3 before it is over-irradiated, and is separated in zone 4 to recover a product that has a surprisingly high V.I. The products obtained by the irradiation can include dry gas, C<sub>4</sub>'s gasoline (0/430), heating oil (430/600), light lube (600/900), bright stock (900/1200), and higher molecular weight polymer.

The irradiated product can be separated in zone 4 in any convenient manner. Distillation is usually sufficient. A product of suitable viscosity and intermediate boiling range is separated and removed by line 5. This intermediate fraction, boiling in the range of 750-950° F., and more preferably 800-875° F., is obtained in yields of about 1 to 20 wt. percent per pass, based on fresh feed, and has a viscosity in the range of 35 to 70, or above, SSU at 210° F., and a viscosity index of at least 120. With recycle operation ultimate yields of over 80 wt. percent are obtained. It has been observed that the concentration of the desired intermediate boiling range fraction builds up to a maximum during recycle of about 12 wt. percent. Beyond this the intermediate fraction appears to be converted to heavier material as fast as it is being formed. For this reason, it is desirable that the recovery of the intermediate fraction be such that its concentration in the feed be substantially below 12 wt. percent.

The material of lower boiling range than the product is removed by line 6. The higher boiling material is removed by line 7. The high V.I. product removed by line 5 can, of course, be further treated by other means in separation zone 4 if desired. Thus, a molecular type separation as dewaxing, extraction of aromatics as by silica gel or solvent treating can be used to separate low V.I. components from the high V.I. product. These low V.I. components of about the same boiling range as the high V.I. product are removed by line 8.

While some of the light material removed by line 6 can be withdrawn as product, preferably a major portion and usually about all of this light material is recycled by line 9 to the irradiation zone to be further converted into the desired high V.I. product. If desired, some of the extremely light components in the material in line 6, i.e., the C<sub>6</sub>-gases, can be removed and discarded.

As will be appreciated by those skilled in the art, better control of the irradiated product can be obtained by recycling a substantial proportion of the irradiated material before such separation. This can be done by line 10. By using recycle, the rate of polymerization and the dosage received by the material is more readily controlled and over-irradiation is easily avoided.

Data also indicates that the product in line 5 can be further increased in viscosity by 5 or more units, with little loss in V.I., by further separately irradiating it in the absence of diluting or contaminating lower or higher boiling components. Thus, in one embodiment of the invention, a portion or all of the product in line 5 is recycled to be separately irradiated by line 11. The conditions here are substantially those used in irradiating the feed material.

The polymer bottoms in line 7 can be disposed of as desired. They are useful as lubricants of the cylinder or bright stock type, and usually have a viscosity at 210° of 150 SSU or better. They can be subject to cracking either thermally, catalytically, or by irradiation as shown by line 12, to recover some of the over-polymerized feed material, and the depolymerized cracked material can be recycled to zone 2 if desired to be again converted, by itself or with fresh feed, into the proper viscosity range material.

If a separation for a low V.I. product be made, then

the material in line 8 can be recycled and further converted either alone with the feed, or can be combined with the contents of line 7 for thermal cracking. In this way the yield of the process is further increased.

#### Example I

600 cc. of substantially pure cetane (n-hexadecane) were irradiated in the Brookhaven National Laboratories atomic pile in a vented aluminum container. The container was maintained at a temperature of 260° F. and at a pressure of about 1 atm. The flux in the container was about  $3 \times 10^{12}$  neutrons per square centimeter per second (n/cm.<sup>2</sup>/sec.), and 1.6 megaroentgens/hour of gamma radiation (1 megaroentgen is equivalent to about  $1 \times 10^{-3}$  kw.h./lb. The irradiation was continued for about 5 days until 300 megaroentgens had been absorbed.

Upon examination of the irradiated material, it was found that the viscosity index reached a maximum at about 40 SSU at 210° F. This irradiated material was separated to obtain a fraction boiling in the range of about 700 to 900° F. This fraction had a viscosity of 38.5 SSU at 210° F., a viscosity index of 145, and a +40° F. pour point. It could be dewaxed to a 0° F. pour by removing 3.5 wt. percent wax and did not break down under shear.

#### Example II

4,362 grams of cetane were passed from a storage drum at a rate of 1500 cc./hr. through an aluminum reactor having an inside diameter of 2 inches and a length of 12 feet. The reactor was located in an unused fuel channel near the center of the Brookhaven pile. The approximate flux was  $0.2 \times 10^{12}$  n./cm.<sup>2</sup>/sec. of fast neutrons,  $1 \times 10^{12}$  n./cm.<sup>2</sup>/sec. of thermal neutrons, and  $1 \times 10^6$  R./hr. of gamma rays. The pressure was about atmospheric and the temperature was 200° to 400° F., varying with the length of the reactor. The material from the reactor was passed through a condenser at 65° F. The liquid product was returned to the storage drum for recycle and the gas was metered and vented. The yields, as weight percent on feed, after 3140 hours of operation were:

|                    |      |
|--------------------|------|
| Gas                | 2.3  |
| 0/430° F.          | 1.5  |
| 430/540° F.        | 3.1  |
| 540/600° F. (feed) | 71.9 |
| 560° F. +          | 21.2 |

Figure II is a plot of the surprising results obtained from the continuous conversion of cetane. The graph gives the viscosity and viscosity index, as the ordinates, of incremental fractions distilled from the irradiated material, the incremental fractions being expressed on the abscissa as being obtained at a certain weight percent distilled off. The 80% point was at 600° F. (atm. eq.), the 90% point was at 835° F., and the 95% point was at 925° F.

This example illustrates the surprising relationship between viscosity and viscosity index of the irradiated material, and shows the unexpected results to be obtained through recycle operation with continuous recovery of a select intermediate boiling range fraction.

Having described this invention, what is sought to be protected by Letters Patent is succinctly set forth in the following claims.

#### What is claimed is:

1. A process comprising irradiating a predominantly paraffinic feed stock boiling in the range of 100 to 700° F. and having a viscosity below 35 SSU at 210° F. with high energy ionizing radiation having an energy level above 30 electron volts, at a rate in the range of 1 to  $50 \times 10^{-3}$  kw. h./lb./hr. and at a temperature up to 700° F., until at least  $5 \times 10^{-3}$  kw. h./lb. of radiation are absorbed, separating the material so irradiated and recovering an intermediate boiling range distillate fraction having a viscosity above 35 SSU at 210° F. and a V.I.

above 120, and recycling a portion of the irradiated material boiling below said intermediate fraction.

2. The process of claim 1 wherein said feed stock contains up to 20 wt. percent of C<sub>1</sub>-C<sub>6</sub> hydrocarbons.

3. The process of claim 1 wherein said intermediate boiling range fraction is further irradiated to increase the viscosity thereof by at least 5 units.

4. The process of claim 1 wherein a portion of the irradiated material is directly recycled before separation, and the recovery of said intermediate boiling range fraction is such that the concentration thereof in the feed is below 12 wt. percent.

5. The process of claim 1 wherein said irradiation is obtained from a nuclear reactor and comprises neutrons and gamma rays.

6. A process comprising irradiating a feed stock boiling in the range of 100 to 700° F. having a viscosity below 35 SSU at 210° F. and comprising at least 75 wt. percent paraffins and under 5 wt. percent aromatics, with high energy ionizing radiation having an energy level above 30 electron volts at a rate in the range of 4 to  $8 \times 10^{-3}$  kw. h./lb./hr. and at a temperature in the range of 300 to 600° F. until 5 to  $600 \times 10^{-3}$  kw. h./lb. of radiation are absorbed, recovering the irradiated mate-

rial, directly recycling to the feed a portion thereof to control in part the degree of conversion, separating the remainder to obtain an intermediate fraction boiling in the range of 800 to 875° F. and having a viscosity in the range of 35 to 75 SSU at 210° F. and a viscosity index of at least 120, and recycling to the feed a major proportion of material from the separation step boiling below said intermediate fraction.

7. The process of claim 6 wherein said high energy radiation is obtained from a nuclear reaction and wherein at least 30% of the energy absorbed by said feed stock is derived from neutrons.

15 **References Cited in the file of this patent**

**UNITED STATES PATENTS**

|            |                  |               |
|------------|------------------|---------------|
| 2,1627,938 | Tingley          | May 10, 1927  |
| 2,350,330  | Remy             | June 6, 1944  |
| 2,516,848  | Brasch           | Aug. 1, 1950  |
| 2,743,223  | McClinton et al. | Apr. 24, 1956 |

**OTHER REFERENCES**

Mincher Knolls Atomic Power Laboratory Report 731, April 2, 1952, pp. 1-8.